

A. Wetherbee,  
Billiard-Cue Tip,  
No 84,036, Patented Nov. 10, 1868.



Witnesses

Samuel P. Farley  
J. S. Colburn

Inventor:

Albert Wetherbee



ALBERT WETHERBEE, OF WALTHAM, MASSACHUSETTS.

Letters Patent No. 84,036, dated November 10, 1868.

**IMPROVED COMPOSITION TIP FOR BILLIARD-CUES.**

The schedule referred to in these Letters Patent and making part of the same.

*To all whom it may concern:*

Be it known that I, ALBERT WETHERBEE, of Waltham, Middlesex county, and State of Massachusetts, have invented a new and improved Tip to be Attached to a Billiard-Cue; and I do hereby declare that the following is a full and exact description of the same, reference being had to the drawings annexed, with letters of reference marked thereon.

The nature of my invention is that of an attachment to the extreme smaller end of a billiard-cue, firmly fastened there, and composed of a combination of substances, of such character as that, friction being created, the tip will not slip upon the ivory billiard-ball when, in the prosecution of the game, it impinges upon it.

In the drawings—

Figure 1 is a side view of my invention.

Figure 2 is a horizontal section of the same.

And in the drawings annexed, A, figs. 1 and 2, is a portion of the smaller end of a billiard-cue.

B, figs. 1 and 2, is the tip which I have invented.

This tip is composed of one-third rubber and sulphur, (the latter in the usual proportion with vulcanized rubber,) and two-thirds of pulverized chalk.

The mode in which I combine these two substances is this: I prefer to use rubber already vulcanized, which I reduce to powder by grinding. With this powder I mix my pulverized chalk, (not confining myself to the exact proportions above named.) The com-

bined substances are then pressed in a mould, and treated by fire, in the usual way.

As is seen in fig. 2, the end of the cue is made concave, the tip being made convex at that side, to fit into it, and secured thereto by glue, shellac, or any convenient cement; but I sometimes have the head of a screw cast into the tip, the screw-portion projecting outward from the tip, and into the end of the cue; and I do not confine myself to any peculiar shape of my tip. Sometimes I make it in the shape of a short cylinder, with the end plane at the side at which it is attached to the cue; and I sometimes make this side of the tip concave, instead of convex. Sometimes I increase the concavity, so that the cue-end of the tip assumes the form of a hollow cylinder, fitting on to the end of the cue.

I do not claim a rubber tip to the end of a billiard-cue; but

What I claim herein as of my own invention, and desire to secure by Letters Patent, is—

A tip of a billiard-cue, made of vulcanized rubber, one part, and pulverized chalk, more than one part, intimately mixed, and baked in combination, all substantially as and for the purpose described.

ALBERT WETHERBEE.

Witnesses:

LEMUEL P. JENKS,  
J. E. COLBURN.